

## UNITED STATES PATENT OFFICE

2,324,123

## FOG INHIBITOR FOR PHOTOGRAPHIC DEVELOPERS

Arnold Weissberger, Rochester, N. Y., assignor to  
Eastman Kodak Company, Rochester, N. Y., a  
corporation of New Jersey

No Drawing. Application July 8, 1941,  
Serial No. 401,439

12 Claims. (Cl. 95—88)

This invention relates to photographic developers and particularly to fog inhibiting or toning agents for developers.

It is well known that fogging occurs in a photographic film or plate when it is developed for unusually long periods of time. It is necessary in most cases to use a relatively weak developer in order to avoid the formation of fog. Soluble bromides, such as potassium bromide, have been used in the developer to overcome this but they do not permit development with a strong developer for long periods of time at temperatures which may go higher than 70° F.

I have discovered that certain derivatives of aminobenzimidazole, for example, 2-amino-6-nitrobenzimidazole and 2-amino-4,6-dinitrobenzimidazole, may be incorporated in the developer to obtain all of these advantages. These compounds may be used either in black-and-white or in color developers. In some cases they may be added to the emulsion or to the subbing or backing layers of the film or plate.

Aminobenzimidazole appears to have one or the other of the following structural formulas:



or



Specific compounds which we have found suitable are 2-amino-6-nitrobenzimidazole and 2-amino-4,6-dinitrobenzimidazole. The structural formula of these compounds, respectively, are as follows, assuming (2) to be the basic formula:



and



2-amino-6-nitrobenzimidazole has previously been prepared by Kym and Ratner, Ber. 45,3254 (1912) however the melting point is given as 189°—190° instead of 245°—246° C. The compounds used in the present invention were prepared by essentially the method of Pierron, Ann. Chem. and Phys. (8), 15, 189—193, by reaction between o-phenylenediamine and cyanogen bromide. 2-amino-6-nitrobenzimidazole nitrate was prepared as follows:

One part of o-phenyleneguanidine was dissolved in about 20 parts of nitric acid (d. 1.42) at room temperature, and the solution allowed to stand at room temperature for 15—20 hours. 15 The bulk of the product crystallized from the reaction mixture during this time. An additional amount was precipitated from the reaction mixture by diluting with 2½ volumes of water. After recrystallization from water the product formed orange-yellow needles which were highly unstable at elevated temperatures. The melting point was about 225° C. The free base melted at 245°—246° C.

In a similar manner other nitro and dinitro, 25 such as the 4-nitro and 4,6-dinitro, derivatives of aminobenzimidazole may be prepared and are contemplated for use in my invention.

The following examples, which are intended to be illustrative only, indicate developing formulas 30 using nitro derivatives of aminobenzimidazole according to my invention.

## Example 1

35 A black and white developer is made as follows:

|                                  |       |    |
|----------------------------------|-------|----|
| Monomethyl-p-aminophenol sulfate | grams | 1  |
| Hydroquinone                     | do    | 5  |
| 40 Sodium sulfite                | do    | 20 |
| Sodium carbonate                 | do    | 30 |
| Sodium hydroxide                 | do    | 1  |
| Water to                         | liter | 1  |

45 On development to a negative for 10 minutes using the above formula a fog density value of 0.40 was obtained. When 1 gram of potassium bromide was added to the developer the fog value fell to 0.18; when the bromide was replaced by 0.25 gram of 2-amino-6-nitrobenzimidazole nitrate the fog value was 0.08. A similar result was obtained with 2-amino-4,6-dinitrobenzimidazole. In the above formula the fog inhibitor of the invention may be used alone or in conjunction with another fog inhibitor such as potassium bromide

## Example 2

60 A developing solution for forming a colored

image by coupler development is made as follows:

A

|                                            |       |    |   |
|--------------------------------------------|-------|----|---|
| 2-amino-5-diethylaminotoluenehydrochloride | grams | 1  | 5 |
| Sodium sulfite                             | do    | 10 |   |
| Sodium carbonate                           | do    | 30 |   |
| Water to                                   | liter | 1  |   |

B

|                                  |       |     |    |
|----------------------------------|-------|-----|----|
| 2,4-dichloro- $\alpha$ -naphthol | grams | 2   | 10 |
| 2-amino-6-nitrobenzimidazole     | do    | 0.2 |    |
| Water to                         | cc    | 100 |    |

In use, B is added to A. This developer produces a blue-green dye on development of an exposed silver halide layer. The amount of aminobenzimidazole derivatives used in either black and white or color developers may vary from about .005 gram to 0.50 gram per liter or higher.

In some cases it may be desirable to develop emulsion layers containing a coupling agent in the emulsion layer, in which case the color-forming developer would contain the fog inhibitors of the invention but would be devoid of coupling agent.

I consider as within my invention all equivalents and modifications falling within the scope of the appended claims.

What I claim is:

1. A photographic developer containing a developing agent and as a fog inhibiting agent a nitro derivative of 2-aminobenzimidazole.
2. A photographic developer containing a developing agent and as a fog inhibiting agent 2-aminobenzimidazole having at least one nitro group on the benzene portion of the molecule.
3. A photographic developer containing a developing agent and as a fog inhibiting agent 2-amino-6-nitrobenzimidazole.
4. A photographic developer containing a developing agent and as a fog inhibiting agent 2-amino-4,6-dinitrobenzimidazole.
5. A color-forming photographic developer

comprising a primary aromatic amino developing agent and a nitro derivative of 2-aminobenzimidazole.

6. A color-forming photographic developer comprising a primary aromatic amino developing agent, a coupler compound, and 2-amino-benzimidazole having at least one nitro group on the benzene portion of the molecule.

7. A color-forming photographic developer comprising a primary aromatic amino developing agent, a coupler compound, and 2-amino-6-nitrobenzimidazole.

8. A color-forming photographic developer comprising a primary aromatic amino developing agent, a coupler compound, and 2-amino-4,6-dinitrobenzimidazole.

9. The method of preventing the formation of fog on development of an exposed silver halide layer, which comprises treating the layer with a developing solution containing a developing agent and a nitro derivative of 2-aminobenzimidazole.

10. The method of preventing the formation of fog on development of an exposed silver halide layer, which comprises treating the layer with a developing solution containing a developing agent and 2-amino-6-nitrobenzimidazole.

11. The method of preventing the formation of fog on color-development of an exposed silver halide layer, which comprises treating the layer with a solution containing a primary aromatic amino developing agent and a nitro derivative of 2-aminobenzimidazole in the presence of a coupler compound.

12. The method of preventing the formation of fog on color-development of an exposed silver halide layer, which comprises treating the layer with a solution containing a primary aromatic amino developing agent and 2-amino-4,6-dinitrobenzimidazole in the presence of a coupler compound.

ARNOLD WEISSBERGER.